

Patented May 11, 1926.

1,584,257

## UNITED STATES PATENT OFFICE.

JIM THOMAS, OF SHREVEPORT, LOUISIANA.

### FURNITURE AND AUTO POLISH.

No Drawing.

Application filed May 26, 1925. Serial No. 33,044.

This invention relates to certain improvements in polishes and has relation more particularly to a polish of this kind especially adapted for use in connection with furniture and the like.

My improved polish comprises the following admixture;—linseed oil, 3 qts., pine rosin, 2 lbs., turpentine, 4 oz., beeswax, 2 oz.

These ingredients after being thoroughly mixed are cooked or boiled for approximately twenty minutes. After cooling, a composition is provided which may be employed to advantage in polishing furniture and the like.

The linseed oil is used to assure a smooth surface and also to harden the other ingredi-

ents employed. The turpentine serves as a dryer and eliminates the liability of a greasy effect when the polish is applied. The beeswax is employed to give a high gloss upon 20 the application of the polish while the pine rosin serves as a binder to hold the other ingredients together after they have been thoroughly mixed and boiled.

I claim:—

A polishing composition comprising a decoction of linseed oil, 3 qts., pine rosin, 2 lbs., turpentine, 4 oz., and beeswax, 2 oz.

In testimony whereof I hereunto affix my signature.

JIM THOMAS.